

# UNITED STATES PATENT OFFICE.

WILLIAM F. SPIES, OF NEW YORK, AND HERBERT D. PEASE, OF RICHMOND HILL, NEW YORK, ASSIGNORS TO LELAND V. SLAUGHT, OF NEW YORK, N. Y.

## DENTIFRICE AND METHOD OF MAKING THE SAME.

1,275,779.

Specification of Letters Patent. Patented Aug. 13, 1918.

No Drawing.

Application filed December 20, 1917. Serial No. 208,068.

*To all whom it may concern:*

Be it known that we, WILLIAM F. SPIES, a citizen of the United States, and resident of New York city, county and State of New York, and HERBERT D. PEASE, a citizen of the United States, and resident of Richmond Hill, county of Queens, and State of New York, have invented certain new and useful Improvements in Dentifrices and Methods 10 of Making the Same, of which the following is a specification.

Our present invention involves as an important factor a new cleansing and absorbent powder peculiarly adapted for cleaning 15 frictionally without abrasion, and also for absorbing and giving off water, medicaments, antiseptics or germicides. Either or both of these qualities may be utilized to great advantage where the powder is used 20 for a dentifrice but the same qualities may be utilized with the same or similar advantages for other cleansing, absorbing, anti-septic or germicidal purposes.

When the powder is used alone its non- 25 abrasive, frictional cleansing properties and ability to absorb and give off fluids are available and where the powder is combined with plastic material to make a tooth paste, or with adhesive binding material to make a 30 tablet, the same desirable qualities are available in combination with others which will be explained hereinafter.

Heretofore tooth powders and pastes have usually contained soap, flavoring extracts, 35 antiseptics or mild germicides, together with a powdered material adapted to have a scouring effect when rubbed upon the teeth. Our experiments show that the precipitated chalk powder commonly used for such purposes acts as an abrasive, the cutting action 40 of which is shown by marked grooves in the teeth when applied to them with brush and water. Any other material having the ability to remove hardened deposit or tartar 45 would also have the ability to abrade the teeth.

As contrasted with this, our invention recognizes that the ordinary tooth brush user should not employ a dentifrice which will 50 do more than prevent or retard the formation of tartar by keeping his teeth free from food and tartar forming secretions; that re-

moving tartar is a special operation for which a dentist should be regularly employed; and that a dentifrice suitable for 55 general use can be and should be free from abrasive substances.

Hence, while our dentifrice may include any or all of the above mentioned ingredients commonly found in ordinary tooth powders and pastes, its novelty and superior qualities result from the novel qualities of the powdered substance which we employ both as regards its use alone and also in combination with soap, antiseptics or germicides. As compared with chalk, its advantageous qualities include a different and superior kind of mechanical cleaning action and a superior and probably different action as an absorber and carrier of the antiseptics, 70 germicides and other ingredients of the dentifrice.

We have discovered and practically demonstrated that solidified, substantially non-structural cellulose powder can be prepared 75 according to methods devised by us so that it will have peculiar frictional qualities whereby when rubbed along the tooth surfaces, the material clings to and effectively cleans the surfaces without abrading them. It takes 80 up mucus and other discharges by absorption and also by adsorption, that is, by clinging to the surfaces of the cellulose. It has a similar non-abrasive cleaning action 85 on metals.

A solidified, substantially non-structural cellulose suitable for our purpose may be prepared in various ways but we prefer only those methods which will result in minute particles of solid, horn-like carbohydrate, preferably one which will be of greater or less hardness according to the percentage of water it contains but in any event, softer than the material to be cleaned thereby, insoluble in water, water absorbent, 90 oil adsorbent and chemically inactive, and resistant in respect to all except the more powerful of the chemical re-agents.

Our preferred method is to make a fine curd-like precipitate from a carbohydrate 100 solution such as fresh, thoroughly converted viscose. This may be accomplished by rendering the solvent non-solvent as by the action of suitable acid salt solutions as for in-

stance, sodium bisulfite or calcium chlorid, or both of them in approximately equal quantities. The cellulose thus freed from solution may be condensed to the desired physical condition by freeing it from some of the admixed water and breaking it up into small particles before it hardens. The precipitate usually contains undesirable impurities which give a yellow color. These 10 impurities are more or less completely removed by repeated washing with water, which may be rendered slightly alkaline by adding a small amount of bicarbonate of soda or equivalent. This is sometimes desirable because of the difficulty in completely removing the acid by the washing and a slight alkaline quality in the product is preferable to the acid quality. The approximately pure product which results from the 20 final washing is dried and ground, preferably to a very fine powder, preferably not less than 100 mesh and usually about 150 to 200 mesh.

In making the powder by the above 25 method, there are certain precautions which should be observed. For instance, poor quality or stale viscose may yield a sort of grape-nut final product instead of the desired horn-like substance. Hence, in order 30 that the viscose cellulose may be certainly obtained of desired freshness and desired quality for our purpose, we prefer to make the process include the making of the viscose as well as the subsequent precipitating 35 of the cellulose hydrate.

The raw material which we use is preferably white paper pulp made from wood by the sulfite process. To one pound of this pulp torn into fine bits, add two pounds 40 of caustic soda dissolved in six pounds of water, let it stand for an hour or so with occasional stirring, press to a dry cake, break up the cake, add eight ounces of carbon disulfid in an air-tight tank, allow the 45 process of conversion into soluble cellulose to continue from two to eight hours. The progress of the reaction may be judged by the successive colors, brown, russet-brown, orange and yellow and by the solubility of 50 the material in water. Over-treatment at this stage of the making of the viscose is to be avoided since it may adversely affect the final product. Since over-treatment does not decrease the solubility, the time to dis- 55 continue the treatment is when repeated solubility tests show that the cellulose has just become fully converted and completely soluble in water. The converted cellulose is then dissolved in thirty pounds of water.

To the resulting viscose solution amounting to forty-six pounds more or less, is added about six ounces of concentrated, say 50% solution of calcium chlorid, and six ounces or more of sodium bisulfite (probably some- 65 what stronger than fifty per cent.). Pref-

erably, these are mixed cold. The effect is to convert the viscose into a thick gelatin-like mass which appears to consist of the cellulose precipitated but not separated, the water in which it was dissolved remaining 70 uniformly diffused and mixed with the cellulose. The same or even better result may be produced by using twelve to fifteen ounces of the sodium bisulfite without the calcium chlorid. The thick gelatin-like 75 product which results in either case may be further thickened in any desired way. One way is to boil it at a low heat with continuous agitation, the result being a smooth, fine mixture from which fine grain 80 particles of the cellulose readily settle out. Another way is to permit the mixture to stand, the cellulose content will then gradually contract, expelling water and with it many of the undesirable impurities. In so 85 doing, it shrinks away from the sides of the container and becomes more and more like solidified gelatin. When the latter stage is reached, the expelled water may be poured off and the gelatin-like mass broken up by 90 hand, or otherwise, to a desired degree of fineness.

The gelatin-like particles produced by either the boiling or the settling method are 95 repeatedly washed and the water strained off through a cloth until the material of the particles are substantially clean.

Washing should be continued for some time after the solution and the substance appear to be clean, a satisfactory degree of 100 cleanliness being determinable by the iodin test. Dilute tincture of iodin, when applied either to the wash water or to the powder either wet or dry, will lose its color if the impurities are still present but will 105 not lose its color if the product has been sufficiently washed.

After final washing, the cellulose particles are dried and ground. Preferably, they are first dried just enough for easy 110 grinding and after grinding, are further dried to the hardness required in the final product. If desired, however, all of the drying may be done before grinding.

The solidified material whether wet or 115 dry is practically clean cellulose which is mainly non-structural and which usually contains more or less water. Though the individual particles are translucent, the powder is almost white with a slight creamy 120 tinge. The particles appear under the microscope as being of more or less irregular structure. Often, there will be visible in the field of the microscope one or more particles of unbroken down fibers. This, like 125 other structural material, will be found lacking in some of the desirable physical and chemical qualities of the non-structural cellulose hydrate, and though we prefer to conduct the process so as to have as little as 130

possible of the structural material, it is nevertheless possible to leave or even to introduce considerable quantities of structural material precipitated in the particles provided it is incorporated with sufficient amounts of the clean, substantially non-structural cellulose hydrate.

Such chemical investigation of the powder as we have made shows that the cellulose powder is relatively stable, neutral and inert, being proof against decomposition from internal reactions and neither dissolved nor attacked by water or alcohol or antiseptics or any of the milder acid or alkaline chemical re-agents.

By conducting the process so that the unremoved calcium content is an appreciable percentage, the substance may be made quite hard, preferably not much harder than the substance of the teeth, for such hardness would result in the abrasive action which is undesirable for dentifrices though it may be desired for other purposes, as for instance, cleaning metal.

In the pure product the hardness and frictional cleaning qualities, as well as the ability of the material to absorb and give off water, antiseptics, germicides and medicaments, and to take up mucus and other mouth secretions, may be varied within a considerable range by varying the water content of the material. In general, the less water the material contains, the harder and more inert it seems to be. While the variability of the material in this respect seems to be more or less uniformly progressive with progressive changes of its water content, it is well to note certain characteristic conditions of the material.

Drying as by exposure to the atmosphere at temperatures, say 80° to 100° centigrade, serves to drive off more or less of the mechanically absorbed moisture, the material retaining some 12% to 15% of water which

appears to be chemically combined in the molecules of the cellulose and so justifying the description of the material as non-structural cellulose hydrate. The water of combination may be driven off, however, and a dehydrated non-structural cellulose produced by continuing the drying for a sufficient time at temperatures up to or slightly above 130° centigrade.

The dehydrated cellulose will chemically recombine with water to produce the cellulose hydrate and the cellulose hydrate will absorb additional water without chemical combination, up to say 40% to 60% of the weight of the material without becoming moist to the touch.

The dry powder either dehydrate, hydrate or moistened hydrate is capable of taking up still further quantities of water by becoming wet, that is by taking up water in film form on the surfaces of the particles and

in the narrow spaces adjacent their points of contact. In this condition, it may be called wet non-structural cellulose. If the powder thus wetted is the dehydrate or the dry hydrate the material of the particles will ultimately absorb enough water to change the material to the fully moistened hydrate.

The powder swells up as it absorbs the water but upon drying it returns to its original state. If the liquid is wholly volatile, it appears to dry to identically the same condition it was in before the wetting, but if the liquid contains non-volatile constituents, they appear to remain chemically unchanged in the pores and on the surface of the particles and become immediately available for their intended purpose as soon as the powder is again moistened.

The above described physical and chemical properties render the powder particularly useful for cleansing or polishing by friction without abrasion and also as a neutral adsorbent and carrier for germicides, antiseptics and medicines. Both qualities are utilized to the fullest extent where the powder is employed for our primary purpose, namely, as the basis for a non-abrasive germicide or antiseptic dentifrice.

Our dentifrice is made by impregnating the finely ground non-structural cellulose powder with the antiseptic germicide or medicament in any desired way, as for instance, by discharging an atomizing spray of the liquid into or over a moving stream of the powder and stirring the latter so as to uniformly distribute the germicide. Desired ingredients may be distributed with more perfect uniformity by diluting them or by wetting or moistening the powder. In either case the impregnated powder may be dried and may be sieved or even reground if necessary to restore the required fineness of grain.

Any suitable germicide or medicament may be used, as for instance, the well known coal tar germicides such as phenols, cresols or xylenols, either with or without a flavoring, odorant or perfuming medium.

The above as well as many other germicides are primarily of an oily nature and may be purchased in the market either in the oily form or in emulsified preparation. The moistening method is suitable for applying the emulsified antiseptics while the dry powder method is more suitable for the oily forms.

The emulsified disinfectants exhibit the greater germ killing power because of the greater availability of small microscopic globules of the relatively insoluble germicide in mixture with water as contrasted with the relatively large droplets of the un-emulsified oil. The emulsified disinfectants may be made with various emulsifying agents.

Soap is the most commonly employed but gelatin, gums and water soluble oils may be employed.

We may employ germicides and antiseptics other than those above named, as for instance, alcohols; also oils that have been impregnated with antiseptics particularly those in gaseous form such as formaldehyde gas dissolved in essential oil, chlorin gas dissolved in paraffin oil; also essential oils such as oil of lavender, bergamot, etc.

Although the word "antiseptic" applies more accurately to material that merely prevents the growth of bacteria without killing them, we elect to use it herein as a generic term to include "germicides" and "disinfectants" which prevent the growth of bacteria because they do kill them.

Our non-structural cellulose powder, though acting perfectly as a frictional cleanser, causes no perceptible abrasion or wear and is a perfect carrier for the germicides and medicaments. Even in a dry state it retains the antiseptic in active condition and when moistened, it readily gives up the antiseptic with its sterilizing qualities unimpaired.

We claim:

1. A frictional cleaning medium comprising finely comminuted non-structural cellulose hydrate.
2. A dentifrice comprising non-structural cellulose hydrate in the form of small, non-abrasive, water absorbent, oil adsorbent particles.
3. A dentifrice comprising non-structural cellulose in the form of small, non-abrasive, water absorbent, oil adsorbent particles impregnated with an antiseptic.
4. A dentifrice comprising non-structural cellulose in the form of small, non-abrasive, water absorbent, oil adsorbent particles impregnated with xylol.
5. A dentifrice comprising finely comminuted particles containing substantially non-structural cellulose impregnated with an emulsified oily antiseptic.
6. A dentifrice comprising finely comminuted particles containing substantially non-structural cellulose impregnated with an emulsified oily disinfectant derived from coal tar.
7. A dentifrice comprising finely comminuted particles containing substantially non-structural cellulose slightly alkaline and impregnated with emulsified xylol.
8. A dentifrice comprising finely comminuted particles containing precipitated, substantially non-structural cellulose impregnated with an emulsified oily antiseptic.
9. A dentifrice comprising finely comminuted particles containing precipitated, substantially non-structural cellulose impregnated with an emulsified oily disinfectant derived from coal tar.

10. A chemically neutral and stable non-structural cellulose hydrate precipitated from viscose solution by action of an acid salt including sodium bisulfite, thoroughly washed while in gelatin-like condition, then further dried and powdered substantially as described. 70

11. A product comprising particles containing solid non-abrasive, water absorbent, oil adsorbent carbo-hydrate impregnated 75 with an emulsified oily antiseptic.

12. A product having antiseptic properties comprising a finely comminuted non-structural cellulose impregnated with an antiseptic. 80

13. A product having antiseptic properties comprising comminuted, substantially non-structural cellulose particles impregnated with an emulsified oily antiseptic.

14. A product having antiseptic properties comprising comminuted, substantially non-structural cellulose particles impregnated with an emulsified oily disinfectant derived from coal tar. 85

15. The method of making a dentifrice powder, comprising a chemically neutral and stable non-structural cellulose hydrate which method consists in subjecting viscose to the action of calcium chlorid and sodium bisulfite, removing water from the resulting gelatin-like cellulose hydrate material, breaking it up, repeatedly washing until neutral under the iodin test, drying until the resultant particles consist of a translucent horn-like substance, then powdering 90 and finally impregnating with an antiseptic. 95

16. The method of making a dentifrice powder comprising translucent horn-like particles of substantially non-structural cellulose hydrate, which method consists in changing viscose to a gelatin-like mass, expelling water from the gelatin-like material and breaking up the mass to form a finely sub-divided precipitate, washing the precipitate to purify the material and render it 100 approximately neutral or slightly alkaline, drying the particles until no longer definitely wet to the touch, and impregnating the material with the desired antiseptic or medicament. 110

17. The method of making particles of precipitated, substantially non-structural cellulose hydrate, which method consists in changing viscose to a gelatin-like mass, expelling water from the gelatin-like material 120 and breaking it up into particles and washing the particles. 115

18. The method of making a dentifrice comprising particles of precipitated, substantially non-structural cellulose hydrate, 125 which method consists in changing viscose to a gelatin-like mass, expelling water from the gelatin-like product to form a finely sub-divided precipitate, washing the precipitate to purify the material and render it ap- 130

proximately neutral or slightly alkaline, drying the particles until no longer definitely wet to the touch, and impregnating the material with an emulsified antiseptic or 5 medicament.

19. The method of making a dentifrice comprising translucent horn-like particles of substantially non-structural cellulose hydrate, which method consists in changing 10 viscose to a gelatin-like mass, dehydrating the jelly-like mass to form a granular or curd-like precipitate, washing the precipitate to purify the material and render it approximately neutral or slightly alkaline, 15 drying, grinding and screening the particles, and compounding the resulting powder

with the other ingredients required to make the desired dentifrice.

20. The method of making a dentifrice comprising particles of substantially non-structural cellulose hydrate, which method consists in changing viscose to a gelatin-like mass, removing water to produce a curd-like finely subdivided precipitate, washing the precipitate and utilizing it as the mechanical cleaning ingredient of the desired dentifrice. 20

Signed at New York city, in the county of New York and State of New York, this 19th day of December, 1917.

WILLIAM F. SPIES.  
HERBERT D. PEASE.